

# UNITED STATES PATENT OFFICE.

JOHN A. KOSOFSKY, OF NEW YORK, N. Y., ASSIGNOR, BY MESNE ASSIGNMENTS, TO  
ETTA KOSOFSKY, OF NEW YORK, N. Y.

## FUR-GLAZE AND THE METHOD OF MANUFACTURING THE SAME.

1,150,208.

Specification of Letters Patent. Patented Aug. 17, 1915.

No Drawing.

Application filed July 12, 1913. Serial No. 778,765.

*To all whom it may concern:*

Be it known that I, JOHN A. KOSOFSKY, a citizen of the United States of America, residing at New York city, in the county 5 and State of New York, have invented certain new and useful Improvements in Fur- Glaze and the Method of Manufacturing the Same, of which the following is a specification.

10 My invention relates to a fur glaze or gloss, and to the method of manufacturing the same.

The gloss, which forms part of my invention, is intended to be applied in liquid 15 form to furs of any kind, for the purpose of imparting luster thereto.

To manufacture one quart of the glaze, I proceed as follows:—To approximately nine-tenths of a quart of water, add one half 20 ounce of naphthalene, stirring the mixture well and thereafter straining the same through a cloth or fine mesh sieve. Then to one tenth of a quart of alcohol add seven drops of oil of rosemary, and add the last 25 named mixture to the water and naphthalene mixture, the whole being well stirred. The glaze which has a very slight odor of naphthalene is then in condition to be ap-

plied to the fur. The glaze may be sprayed onto the fur, or applied thereto in any other 30 suitable manner.

I find, in practice, that by the use of the glaze above described, a natural gloss may be imparted to old and worn furs, giving them the appearance of new furs. 35

Having described my invention, what I claim as new and desire to secure by Letters Patent is:—

1. A fur glaze, comprising water, alcohol, a trace of naphthalene, and odorous oil essence, substantially as described. 40

2. A fur glaze, comprising nine-tenth parts of water, one-tenth part of alcohol, a trace of naphthalene, and oil of rosemary. 45

3. The herein described method of manufacturing fur glaze, which consists in admixing water and naphthalene, straining the mixture, and thereafter adding thereto a mixture of alcohol and oil of rosemary. 50

In testimony whereof I have affixed my signature in presence of two witnesses.

JOHN A. KOSOFSKY.

Witnesses:

ALFRED H. LANG,  
Wm. J. ELLINGSEN.

Copies of this patent may be obtained for five cents each, by addressing the "Commissioner of Patents, Washington, D. C."